

(Specimens.)

F. J. SEYMOUR.

PROCESS OF OBTAINING ALUMINIUM.

No. 291,631.

Patented Jan. 8, 1884.

Fig. 1.



Fig. 3.



Fig. 2.

Witnesses:  
Ed L. Moran  
Geo. Wadman

Inventor:  
Frederick J. Seymour  
by his Attorneys  
Brown & Brown

# UNITED STATES PATENT OFFICE.

FREDERICK J. SEYMOUR, OF WOLCOTTVILLE, CONNECTICUT, ASSIGNOR OF ONE-HALF TO WILLIAM HENRY BROWN, OF NEW YORK, N. Y.

## PROCESS OF OBTAINING ALUMINIUM.

SPECIFICATION forming part of Letters Patent No. 291,631, dated January 8, 1884.

Application filed September 17, 1883. (Specimens.)

*To all whom it may concern:*

Be it known that I, FREDERICK J. SEYMOUR, of Wolcottville, in the county of Litchfield and State of Connecticut, have invented 5 a new and useful Improvement in Processes of Obtaining Aluminium from Aluminous Ores and Earths, of which the following is a specification.

The natural condition in which aluminium is found most abundant is in the kaolin clays. Aluminium is also found in refractory ores carrying other metals, as nickel, cobalt, copper, zinc, and iron. Operations by heat in open furnaces or vessels will fail to cast down 15 into a metallic state zinc and aluminium, as, owing to their volatile nature, they are resolved into vapor and driven off; but either may be obtained by mixing the ore or earth which contains it with carbonaceous material 20 and subjecting the mixture to heat in a close retort.

I have ascertained that the casting down of the aluminium in the metallic condition in the retort is very greatly expedited by the presence of zinc, the aluminium and the zinc having a great affinity for each other, and the latter serving as a flux to the former; and my invention consists in mixing aluminous ores or earths with ores of zinc and with carbonaceous matter, and in subjecting the mixture to heat in a close retort. In this way I obtain in the retort an alloy of zinc and aluminium which may be useful for some purposes, as for mixing with other metals or alloys, or which may be afterward treated to separate the aluminium from the zinc when it is desired to obtain the aluminium in a pure or nearly pure state. 30

The aluminous ores and earths which may be treated by this process are various; but 40 that with which I have most successfully operated is the kaolin, which is found in great abundance in South Carolina, and the ores of zinc which I have used in my process are the calamine ores found in Missouri and New Jersey.

In the accompanying drawings, Figure 1 is a vertical section of a retort-furnace to be used in carrying out my improvement. Fig. 2 is a longitudinal section of one of the retorts upon 50 a larger scale, and Fig. 3 is a vertical section

of a machine for separating the aluminium from the zinc with which it is obtained.

Similar letters of reference designate corresponding parts in all the figures.

A is the furnace-chamber. B is the grate. C D are the furnace and ash-pit doors, and E is the chimney. In this furnace are arranged any desired number of retorts, F, which are shown as closed at one end and provided at the outer end with removable stoppers or heads F'. These retorts may be made of iron, 55 clay, or other suitable material, and are here shown as supported in the front wall of the retort-furnace and on bearers or string-pieces A', extending across the furnace. These retorts are removable from the furnace-chamber for the purpose of filling them.

Referring now to the apparatus shown in Fig. 3, and which is similar to that forming the subject of my Patent No. 199,475, dated January 22, 1878, except that the vessel G, for containing the molten metals, is closed, this vessel may be made of iron or other suitable material, and is mounted on a vertical shaft, and rotated through bevel-wheels a by a driving-shaft, I, which may be driven by a belt or otherwise. As the vessel is rotated it is subjected to a jiggling or up-and-down motion by a cam, b, on the shaft acting on a stationary cam, b', at the step-bearing of the shaft. The vessel G is arranged in a heating-chamber, J, which may be heated by a furnace, (not here shown,) but which may be arranged as shown in my former patent. 75

At the top of the chamber G is a chimney, J'.

In the top of the vessel G is an inlet-aperture, closed by a cover, c, which may be luted or otherwise made air-tight, and in the side of the vessel are tapping holes d d' d'' d''' at different levels. 90

K is a delivery-spout, whereby the molten metal is carried outside the chamber, and J'' is an opening, through which access may be had to the tapping-holes d d' d'', &c. It is closed by a door, J'.

As here shown, the cover c and mouth of the vessel G are accessible through a door, e, in the chimney J'; but they might be accessible through a hole in the top of the chamber J. 95

I will now proceed to describe the operation of my invention. The zinc ore is first prepared by roasting to expel the sulphur, and the kaolin or aluminous ore is dried. 5 Both are pulverized, and then mixed with pulverized solid carbonaceous matter, and a proper quantity of a suitable flux is added. The carbonaceous matter should be nearly pure carbon. That which I have successfully used consists of equal parts bituminous coal and willow-charcoal. The flux which I have used is common salt. The proportions of the several materials with which I have obtained the best results are as follows, by weight: kaolin, sixty 10 (60) parts; zinc-ore, sixty (60) parts; carbonaceous matter, one hundred and twenty (120) parts; common salt, three (3) parts. These materials having been thoroughly mixed, I pack the mixture into the retorts F, which 15 have been coated or luted internally, and after closing and sealing the stoppers or heads F', I subject the retorts and their contents to the proper degree of heat in the furnace A. The combined action of the heat, the carbon, and 20 the fluxes will cast down nearly all the zinc and aluminium contained in the ores, and when the metals will flow freely they are drawn off. The alloy of aluminium and zinc thus obtained may be allowed to cool for further treatment 25 or use; but if the metals are to be separated it is at once introduced into the vessel G, which is also properly coated on its inner surface. The vessel or retort G is then closed, and its cover is sealed or luted. This vessel or retort is so arranged that it may be subjected to 30 a variable and determinable heat under perfect control, and when the contained metal is at the desired heat a rotary motion is given to the vessel or retort and its contents. As 35 the vessel is rotated it also receives a jiggling action by means of the cams b b'.

As the melting-point of zinc is about seven hundred and forty degrees ( $740^{\circ}$ ) and that of aluminium is about eight hundred and forty, 45 ( $840^{\circ}$ ), and as zinc begins to crystallize at about five hundred and sixty degrees, ( $560^{\circ}$ ), it follows that the great difference in the character of the two metals as to their point of crystallization and the great difference in their specific 50 gravities will enable an almost perfect separation of the aluminium and zinc to be made. After the agitation of the molten metal has been continued for a time, it will be found that by tapping the lower holes, d or d', zinc will 55 be obtained, while by tapping the upper holes, d' d', aluminium will be obtained. The pro-

cess of separation may be continuous, so that if the zinc after the treatment still carries some proportion of aluminium, additional mixed metals are added and the process continued. 60 An alloy of zinc and aluminium in uncertain proportions may be drawn from the retort G during the first stages of the process, and this alloy will have commercial value, as it will be useful to alloy with copper, zinc, and nickel. 65

It will be understood that by my invention I can obtain aluminium either in a substantially pure state or as an alloy with other metals.

I am aware that it is not new to use metallic zinc for the purpose of extracting aluminium from a heated spongy mass of aluminium and carbon which has been obtained previously by heating alumina with a liquid hydrocarbon, as that is described in English Patent No. 2,137, 70 A. D. 1868; but my process differs from that, in that I extract the aluminium from aluminous earth or ore by the use of an ore of zinc at one operation, while that involves two operations to accomplish by the use of metallic 75 zinc what I do in one by the use of the zinc ore.

I am also aware that it was proposed in the said English patent to obtain alloys of aluminium by mixing the respective metallic oxides 80 with gas-tar and heating the mixture in a retort; but there is no mention in said patent as to what are the metals with which the aluminium is to be thus alloyed, and it does not therein appear that the oxide which was to be 85 used besides the oxide of aluminium could serve or was intended to serve the purpose of casting down the aluminium in the retort in a metallic state, which is what I effect by using the ore of zinc in the retort with the aluminous 90 earth or ore.

What I claim as my invention, and desire to secure by Letters Patent, is—

The improvement in the art of extracting aluminium from aluminous earths and ores, consisting in mixing aluminous ore or earth and an ore of zinc with carbonaceous material and a flux, and subjecting the mixture to heat in a close retort, whereby the zinc liberated is caused to produce or assist in the casting down 100 of the aluminium in a metallic state, and an alloy of zinc and aluminium is obtained, substantially as herein described.

FREDERICK J. SEYMOUR.

Witnesses:

EDW. L. FRISBIE, Jr.,  
W. H. WETHERELL.